

May 8, 1956

A. C. HUTCHISON

2,744,816

SOLID GAS-GENERATING CHARGES

Filed Aug. 11, 1953

Fig. 1



Fig. 2



INVENTOR.  
ALEXANDER CANTLAY HUTCHISON

BY *Raymond C. Leonard*  
*his attorney*

# United States Patent Office

2,744,816

Patented May 8, 1956

1

2,744,816

## SOLID GAS-GENERATING CHARGES

Alexander Cantlay Hutchison, Saltcoats, Scotland, assignor to Imperial Chemical Industries Limited, a corporation of Great Britain

Application August 11, 1953, Serial No. 373,498

Claims priority, application Great Britain  
October 10, 1947

23 Claims. (Cl. 52—5)

This invention relates to improvements in solid gas-generating charges. More particularly, it relates to charges of the relatively slow-burning kind capable of propagating through themselves a self-sustaining exothermic non-detonating gas-evolving decomposition when a merely local portion of the charge is heated from room temperature to the temperature at which its active decomposition begins. Such gas-generating charges have found application heretofore for a variety of purposes including, for instance, the actuation of gas pressure operated mechanical devices, safety (flameless) blasting operations, the dispersion of volatilizable pesticides, insect repellants and rodenticides, propulsion of rockets and the expulsion of liquids from containers such as fire extinguishers.

In accordance with the present invention, gas-generating charge compositions of the foregoing general type and scope of utility are provided which, however, are characterized and distinguished essentially by the fact that they consist in major part of guanidine nitrate, together with a polynitro-phenol or a polynitroso-phenol in proportion which may vary considerably but is always much less than one-half that of the guanidine nitrate component. The charge compositions of the invention are non-explosive and are not capable of being detonated by a blasting cap or other form of commercial detonator. Accordingly, they are to be sharply distinguished from compositions such, for example, as smokeless powders, and conventional blasting compositions which are essentially detonating explosives having a base of nitrocellulose, of nitrocellulose and nitroglycerin, or of oxidizing salts, but which may sometimes include guanidine nitrate as an incidental component.

It is known that guanidine nitrate undergoes an exothermic gas-evolving decomposition when it is strongly heated, but under atmospheric pressure conditions the reaction does not sustain itself if a portion only of a quantity of the compound is heated from atmospheric temperature to the temperature at which decomposition begins, unless external heating is maintained. The decomposition leads to the production of steam, nitrogen, ammonia and oxides of carbon, but there is also formed a certain amount of a difficultly fusible yellow nitrogenous organic residue.

When the conditions are such that the prevailing gas pressure is sufficiently high, namely of the order of 70 atmospheres, once the reaction has been locally initiated it will sustain itself throughout a mass of the guanidine nitrate, and under such gas pressure conditions the products are almost wholly gases and vapors.

It has been proposed to provide mixtures containing guanidine nitrate charges that are capable of decomposing with a high yield of permanent gases when locally heated by a non-detonating element at a lower pressure than is required for guanidine nitrate alone, said mixtures comprising guanidine nitrate with a proportion of a metallic hypophosphite or ammonium hypophosphite where-

2

by there may be obtained, if desired, charges capable of self-sustained decomposition even at atmospheric pressure when locally heated.

Owing to the nature or amount of the residue the hypophosphites leave behind or because of other disadvantages attendant on their employment, these previously proposed charges have only a limited applicability. Hence it would be desirable to provide improved gas-generating charges based on guanidine nitrate and capable of self-sustained decomposition under conditions of much lower gas pressure than guanidine nitrate alone.

It is also known that the pressure required to render possible the self-sustained decomposition of a charge based on guanidine nitrate may be progressively reduced by making up the guanidine nitrate into charges with progressively increasing amounts of colloided nitrocellulose as a binding agent, by mixing the guanidine nitrate with a solution of nitrocellulose in a volatile solvent, forming the resulting paste into the required shape and evaporating off the volatile solvent. However, the use of a volatile solvent adds to the expense and necessitates a drying operation, while the applicability of this method is also somewhat limited.

I have now found that non-explosive gas-generating charges based on guanidine nitrate, suitable for a variety of purposes and free from the disadvantages attendant on the use of hypophosphites or gelatinized nitrocellulose, and capable of self-sustained non-detonating decomposition when merely locally heated, with a high yield of hot gases at relatively low pressure, considerably lower than the 70 atmospheres required for guanidine nitrate alone, may be obtained by the use in admixture with guanidine nitrate of a polynitro-phenol or a polynitroso-phenol, i. e. a phenol which contains in addition to at least one phenol hydroxyl group a plurality of substituent groups each consisting of a nitrogen atom attached exclusively to at least one terminal oxygen atom and to one of the nuclear carbon atoms of the phenol. While no commitment is here intended as to the mechanism of the action or reaction whereby thermal decomposition of the guanidine nitrate at atmospheric or relatively low superatmospheric pressures is facilitated by the admixed polynitro-phenol or polynitroso-phenol, such admixed compound is conveniently referred to as a sensitizer for such thermal decomposition. The sensitizing action of the particular class of compounds employed for this purpose in the present invention is not general but appears to be specific to guanidine nitrate. Thus, contrary to what might be expected from their action on guanidine nitrate, it has been found that a compound of this class has substantially no heat-sensitizing action on nitro-guanidine, for example. Incidentally, it is to be noted that nitro-guanidine is an explosive, whereas guanidine nitrate is not.

Among the many polynitro- and polynitroso- derivatives of phenol that can be employed as thermal decomposition sensitizers in practicing the present invention, the following may be mentioned by way of example: 2:4 dinitro-resorcinol, 2:4:6 trinitro-resorcinol, 2:4 dinitroso-resorcinol, 4:6 dinitro-ortho-cresol, 3:5 dinitro-catechol, 2:6 dinitro-paracresol, and 3:5 dinitro-salicylic acid. Of these, 2:4 dinitro-resorcinol works particularly well and is presently regarded as most desirable.

With regard to the proportion of polynitro-phenol or polynitroso-phenol sensitizer to be employed in the novel charges of the invention, this may vary widely depending upon such factors as the specific purpose and consequently the specific nature of the charge composition, and the conditions (particularly the pressure) under which the relatively slow, gas-generating thermal decomposition is intended to take place. The limiting considerations are (1) that enough sensitizer must be employed to ensure

occurrence of the desired self-sustaining decomposition; and (2) that the proportion must not be so high as to render such decomposition explosive or detonating in character.

Thus, assuming the charge composition not to include what can properly be termed a "diluent," i. e. an ingredient which merely absorbs heat supplied by the aforesaid self-sustaining exothermic decomposition, and further assuming that the decomposition, once it is initiated by localized heating of the charge, is to be self-sustaining under relatively low working pressures, e. g. from superatmospheric pressures around 10 atmospheres down even to ordinary atmospheric pressure, a proportion of the aforesaid sensitizer ranging from about 8 to about 20 per cent of the weight of the guanidine nitrate ordinarily suffices to render the composition capable of self-sustained decomposition, the proportion being permissibly less as the intended working pressure increases.

Where the working pressure conditions contemplated for self-sustained, non-detonating, exothermic decomposition of the charge are of an order of magnitude higher than about 10 atmospheres, and again assuming substantial absence of diluent or heat-absorbing ingredients, the proportion of the polynitro-phenol or polynitroso-phenol sensitizer component may of course be reduced below the above-indicated minimum. In some instances, it may even be as low as 3 per cent of the weight of the guanidine nitrate, although for optimum performance it is seldom desirable that less than about 5 per cent of said weight be employed.

On the other hand, where the charge does include diluent or heat-absorbing material such, for example, as a smoke-forming agent, a pesticide or other filler which it may be desired to disperse with minimum decomposition thereof, it is frequently necessary or desirable to employ a larger proportion of the aforesaid sensitizer component than the above-indicated maximum of 20 per cent, based on the weight of the guanidine nitrate, in order to ensure satisfactory self-sustained exothermic decomposition of the latter, especially under the working conditions of relatively low temperature and pressure most advantageously characterizing utilization of such diluted charge compositions. However, the fundamental consideration that the gas-generating charge compositions of the invention must be non-explosive and non-detonating in their exothermic decomposition imposes a positive upper limit upon the proportion of polynitro- or polynitroso-phenol derivative permissible to employ therein. Since some of these derivatives (e. g. dinitroresorcinol) are themselves explosives, the higher the proportion of such explosive derivative present in the charge composition, the greater the possibility that said composition may approach being explosive or detonatable, especially if the charge also includes ammonium nitrate or ammonium perchlorate in the restricted small proportions which, as will presently appear, may be desirable and permissible to employ in some circumstances. Generally speaking, therefore, it is desirable to keep the proportion of the phenol sensitizer down low enough to exclude that possibility. Accordingly said proportion should in no event exceed 35 per cent of the weight of the guanidine nitrate at the most, even in the absence of oxidizing salts like ammonium nitrate or perchlorate, and it is generally better practice to hold it down to not substantially above 30 per cent.

If desired, the charges according to the invention may include an aliphatic carboxylic acid selected from the group consisting of tartaric, maleic, citric and fumaric acids. The presence of an aliphatic carboxylic acid permits less of the polynitro-phenol or polynitroso-phenol to be present. This is because the aliphatic carboxylic acids are in fact sensitizing agents for the decomposition of guanidine nitrate. Being cheaper than the polynitro- and polynitroso-phenols, they can therefore sometimes be used

with advantage to replace a portion of the phenol derivative sensitizer. But since these carboxylic acids are less powerful sensitizers than the phenol derivatives aforesaid, it is not desirable to carry such replacement so far that the gas-generating decomposition rate of the charge composition may become too slow. In general, it may be taken that one part of dinitroresorcinol (e. g.) is equivalent, in so far as it can be equivalent, to two parts of tartaric acid (e. g.). It is accordingly evident that, judiciously employed, the aliphatic carboxylic acids provide a means for adjusting or controlling the gas-generating decomposition of the novel charge compositions within reasonable limits, as may be desired. However, the use of such a carboxylic acid in proportion substantially exceeding about 10 per cent of the weight of the guanidine nitrate is not ordinarily to be recommended for best results.

When charges made up only from guanidine nitrate and a polynitro-phenol or polynitroso-phenol are consumed under atmospheric pressure conditions, or at comparatively low superatmospheric working pressures e. g. up to about 10 atmospheres, their decomposition into gaseous products is not quite complete, and they leave a certain amount (usually 15 to 20%), of the difficultly fusible nitrogenous organic residue already referred to. At such pressures, moreover, the generated gases contain appreciable quantities of vaporized condensable organic materials, the presence of which may be undesirable in certain applications of the charges e. g. if they are to be used as power gases in driving engines or operating other mechanical devices where these organic vapors can condense and cause fouling of pipes or moving parts.

It is found however that the inclusion of a small proportion of a promoter, such as vanadium pentoxide, amounting for example to about 0.2 to 1 per cent of the weight of the guanidine nitrate, has the effect of completing the decomposition of the guanidine nitrate, thus obviating the formation of the aforesaid yellow difficulty fusible organic residue and correspondingly increasing the yield of hot gases at working pressures at which this residue would otherwise be formed; and, especially where power gases are to be produced, it is therefore best to include in the charge a small proportion of vanadium pentoxide or of a chemically equivalent vanadium compound decomposable on heating to yield a vanadium oxide, such for example as ammonium vanadate. Vanadium tetroxide may also be used. It has also been found that metallic molybdenum or a compound of molybdenum, e. g. molybdic acid, molybdic oxide, ammonium molybdate, may be used in place of a vanadium compound as a promoter or catalyst for the same purpose. These materials, or the residual thermal decomposition products thereof, as well as the surface contact materials to be presently mentioned, may be broadly termed non-volatile heat-resistant materials capable of acting catalytically to promote maximum production of gases in the self-sustaining decomposition of the charge.

It has further been found that the condensable vaporized organic compounds that would otherwise be formed at atmospheric or relatively low superatmospheric pressure and carried off by the hot gases can be destroyed by causing them to undergo an exothermic reaction while in mixture with the gases proper, in the presence of catalytic surface contact material, whereby at the same time the total hot gas yield is increased. This may be done by causing the mixture of gases and vapors, before cooling takes place, to pass over suitable heat-resisting catalytic solid surfaces that are filamentary in character, such as those of iron, steel or platinum wire gauze, or asbestos, which are herein generically designated as gas-permeable bodies of refractory material; or by including in the composition of the charge a small percentage of asbestos fibre or other heat-resisting material characterized by a large surface and amounting usually to not less than about 0.25% nor substantially more, ordinarily, than

about 2%. When such large-surface refractory material is actually incorporated in the charge, the proportion thereof should of course be kept down to a minimum consistent with effective action. So employed, it also steadies the self-supporting characteristics of the reaction and holds together the ash of the charge. It may be desirable to include a small percentage of potassium nitrate in the charge amounting, for instance, to about 0.25 to 1% thereof, since the potassium nitrate assists the reaction between the gases and vapors on the solid catalytic surface. The use of the potassium nitrate is especially desirable if the charge is in an unusually cold condition before it is locally ignited, or in an environment such that the gases and vapors are at a lower temperature than that at which they would normally be generated. Using as much as 5% potassium nitrate is permissible, but is virtually never necessary. Therefore since it would increase the quantity of residual slag and also correspondingly reduce the proportion of guanidine nitrate in the charge, the use of as much as 5% is virtually never resorted to in practice.

Charges made in accordance with the invention may be used for instance for actuating gas pressure operated mechanical devices, e. g. for driving engines, or for operating pneumatic tools, for operating fire extinguishers, for propulsion of rockets and other gas escape reaction propelled devices, for dispersing insecticidal or the like substances, for making colored smokes, or for safety blasting operations by means of blasting assemblies in which the charge is caused to undergo decomposition in a pressure resisting container adapted to vent the gases once a predetermined pressure has been built up within the container. It will be understood that according to the purpose for which the charge is required it may be in powder, granular or compact form of any required shape, and may or may not include ingredients for reducing or raising the temperature of the gases it generates. The hereinafter mentioned thermally volatilizable fumigating or smoke producing materials are examples of ingredients which reduce the temperature of the said gases and, by way of example, ammonium perchlorate and ammonium nitrate are reagents which raise the temperature of the said gases.

Where charges embodying the invention are not for power-gas production but include insecticidal or other substances to be dispersed, such substances may be thermally volatilizable materials as, for instance, insect repellants, insecticides, fungicides, bactericides and other pesticides; as well as smoke-producing compounds, including colored dyestuffs. In this case the charge will usually be required to decompose under atmospheric pressure conditions. Moreover, if any of the aforesaid materials is an organic compound it will be understood that, if the charge is to include asbestos fibre or other material of large-surface characteristics, such surface-contact material must be employed in such manner that the gases and vapors will not undergo to any extent a reaction on its surface so intense as to destroy a large proportion of the volatilizable compound in the gas stream. The volatilization of the organic compound has in itself a cooling effect so that if sufficient of such compound is used the temperature will be too low for any such undesirably intense surface reaction to take place. For example, 4:6 dinitro-ortho-cresol is a polynitro-phenol that has itself marked insecticidal and arachnicidal properties, a fact which may be taken advantage of to a certain extent if the charge contains an excess of the amount of this polynitro-phenol over that recommended hereinbefore for a charge to be used solely for power-gas generating purposes. When an excess of this material is present, not all of it will be decomposed by the gas producing reaction and the excess will be volatilized and available for effecting fumigation. Normally, however, it is considered preferable to incorporate a specific reagent, such as "DDT" or "Gammexane" as illustrated

in certain of the following examples, for producing a fumigating device of the type proposed. Generally speaking, the amount of insecticidal or other volatilizable or dispersible material thus included in the charge should not materially exceed about 20 per cent by weight of the entire charge.

Another way of reducing the temperature of the gases generated by the guanidine nitrate decomposition is to include in the charge a small proportion, not exceeding about 10 per cent, of a carbonate, e. g. calcium carbonate, decomposable at the temperatures involved, e. g. on the order of 1000° C. The amount of such inclusion should ordinarily not exceed about 10 per cent of the charge as a maximum.

Where, on the other hand, it may be desired to increase the temperature of the evolved gases above what it would otherwise be, minor proportions of an oxidizing salt, such as ammonium nitrate or ammonium perchlorate, may be included, but always with due care that the charge composition shall nevertheless remain non-explosive and non-detonating in character. Thus the charge may safely include up to 20 per cent ammonium nitrate, or up to 10 per cent ammonium perchlorate, provided that with these maximum proportions the charge does not contain more than about 10 per cent of the polynitro- or polynitroso-phenol, and provided the mixture is compressed to a density of not less than 1.4 cc. per gram.

In order to make still clearer the principles underlying the invention, typical desirable embodiments thereof are illustrated hereinafter by means of specific examples, certain of said examples including structural details of gas-generating charge arrangements which are desirable practically and which are further illustrated in the accompanying drawings, wherein

Fig. 1 is a cross section in elevation of one type of cartridge containing a charge embodying the invention; and

Fig. 2 is a cross section in elevation of another type of cartridge illustrating a typical use of a slightly modified charge.

In the aforesaid specific examples now to be set forth, it is to be understood that the stated percentages are by weight.

#### Example 1

In this instance, the charge composition is intended primarily for production of power-gases, with virtually complete decomposition of the guanidine nitrate base, and substantial absence from the gases of organic material condensable in the apparatus utilizing said gases. To this end, a mixture of the composition:

|                        | Percent |
|------------------------|---------|
| Guanidine nitrate      | 88.75   |
| 2:4 dinitro-resorcinol | 10.0    |
| Asbestos fibre         | 0.5     |
| Vanadium pentoxide     | 0.5     |
| Potassium nitrate      | 0.25    |

is subjected to ball milling until the composition is well mixed and pulverized. 3 lbs. of the mixture is then loaded in four equal increments into a 3" diameter open-ended steel tube 10 lined with compressed asbestos fibre sheeting 11, as illustrated in Fig. 1, each increment being pressed for 1 minute at 7000 lb. per square inch, the compressed composition 12 occupying all but one inch at each end of the length of the tube. A hole 13 of 1 inch diameter is then drilled axially through the length of the compressed composition. Four or five circular disks 14 of iron wire gauze, each of 3" diameter and of a mesh ranging from 10 to 50 to the inch (BSS) are fitted into one end of the tube and an electrical ignition system, indicated generally at 15, including a rod of cordite 16 weighing 20 grams, is arranged at the other end of the tube with the cordite extending into the drilled channel 13.

The tube containing the composition is used to operate

a motor of rotary blower design at a progressively increasing speed at a constant working pressure of about 120 lbs. per square inch. The charge leaves an incombustible skeleton amounting to less than 1.25% of the weight thereof, without depositing any condensed organic material in the apparatus.

*Example 2*

In this case also, production of power gases substantially free from condensable components is the objective. A 10 mixture of the composition:

|                        | Percent |
|------------------------|---------|
| Guanidine nitrate      | 88.7    |
| 2:4 dinitro-resorcinol | 9.8     |
| Potassium nitrate      | 0.25    |
| Vanadium pentoxide     | 0.5     |
| Mineral oil            | 0.5     |
| Asbestos fibre         | 0.25    |

is subjected to ball mixing until the ingredients are well mixed into the form of a fine powder. 20 grams of the mixture are pressed in a tubular mould 0.95 inch in diameter lined with asbestos paper under a pressure sufficient to give a well consolidated pellet. In this instance, as shown in Fig. 2, the pellet 20 with its asbestos sheath 21 is ejected from the mould and fitted into a cylindrical container (not shown) of approximately 1" diameter closed at one end and fitted with a screw-on cap at the other end carrying a jet 0.055 inch in diameter. The ignition system, indicated generally at 22, for the pellet at the open end consists of a sliver of cordite 23 held on the surface of the composition by means of a tightly fitting circular disk of 60-mesh BSS stainless steel wire cloth 24 with a length of thin black-powder fuse 25 running from the cordite to the exterior through the jet in the cap of the container.

This miniature jet motor forms the propulsion unit of a model racing car. The ignition is brought about by igniting the fuse with a match which ignites the cordite, which in turn locally heats the composition of the charge to the temperature at which the evolution of the gases becomes active, the decomposition then sustaining itself through the charge. In this manner a thrust of 3 oz. weight lasting for 20 seconds is exerted on the model racing car. The ash is a coherent skeleton of the pellet and amounts to about 1% of its weight.

*Example 3*

The specific embodiment of the invention to which this present example is directed, like those illustrated in the succeeding examples as well, differs from those of Examples 1 and 2 primarily in that a diluent material that is to be dispersed as such, in this instance an insecticide or an insectifuge, is a substantial component of the mixture; and that self-sustained decomposition of the guanidine nitrate at ordinary atmospheric pressure is desired. With this in view, a mixture of the composition:

|                                                                          | Percent |
|--------------------------------------------------------------------------|---------|
| Guanidine nitrate                                                        | 67      |
| 4:6 dinitro-o-cresol                                                     | 18      |
| Alpha-alpha-bis-(parachloro-phenyl)-beta-beta-beta-trichloroethane (DDT) | 15      |

is prepared by grinding the ingredients together until they are well mixed in the form of a fine powder. 20 grams of the mixture are consolidated into the form of a pellet 1 inch in diameter by compression in a mold and ejected. The resulting insecticidal pellet when strongly heated at one end, e. g. by the flame of a Bunsen burner or by means of an ignition composition, supports its own decomposition, giving a yellow smoke without flame, containing most of the DDT as well as some undecomposed excess of 4:6 dinitro-o-cresol, which latter itself also has insecticidal properties as noted hereinabove. This smoke deposits a fine coating of insecticidal material on surfaces

contacted by it, thus rendering them lethal to house flies (e. g.) for some time. The pellet leaves a non-volatile residue amounting to about 10% of its weight. In this example, because of the diluting and heat-absorbing effect of the added specific insecticide ingredient that is to be dispersed by thermal decomposition of the charge proper, with resultant cooling of the generated gases, the polynitrophenyl is employed in much larger proportion than in Examples 1 and 2. Thus, in the present example, the quantity of this material employed amounts to 26.3% by weight of the guanidine nitrate which latter, however, still remains the greatly preponderating or major ingredient of said charge. The 10% residue left by the pellet consists in part of the before-mentioned difficultly fusible yellow-nitrogenous organic material, due to omission from this charge of vanadium pentoxide or an equivalent promoter necessary to ensure complete decomposition of the guanidine nitrate at atmospheric pressure. The omission also of asbestos or other large-surface heat-resistant contact materials from this type of charge has the advantage of permitting a larger proportion of the organic insecticidal material carried by the generated gases to escape destructive decomposition and to perform its intended function.

*Example 4*

In this example, the purpose and ingredients of the charge are substantially the same as in Example 3, except that the gamma-isomer of hexa-chloro-cyclohexane (Gammexane) is substituted for DDT. An insecticidal pellet is prepared from the resulting mixture and its decomposition is initiated after the fashion described in Example 2. Its decomposition produces a yellow smoke without flame, containing 4:6 dinitro-o-cresol and 35 Gammexane which deposits a fine coating of powder 35 lethal to house flies. The non-volatile residue again amounts to about 10% of the weight of the pellet.

*Example 5*

A mixture of the composition:

|                      | Per cent |
|----------------------|----------|
| Guanidine nitrate    | 65       |
| Dinitroso-resorcinol | 15       |
| Gammexane            | 20       |

is ground thoroughly until mixed in the form of a fine powder. In this case, the proportion of polynitroso-phenol sensitizing agent employed is approximately 23 per cent of the weight of the guanidine nitrate.

A 20 gram insecticide pellet of the composition is 50 pressed as described in Example 3 and its decomposition is initiated in similar fashion. A dense white smoke containing Gammexane is produced without any flame. Here also, the non-volatile residue amounts to about 10% of the weight of the pellet.

From the foregoing it is apparent that, in accordance with the present invention, a gas-generating charge embodying the invention consists in major part, most desirably at least 60 per cent, of guanidine nitrate heat-sensitized by a variable but always much smaller quantity of a phenol of the character specified, never exceeding 35 per cent by weight of the guanidine nitrate and being usually less than 30 per cent thereof; also that said charge may include the hereinabove indicated small percentages of decomposition-assisting or catalyzing agents 65 adapted to promote maximum gas yield and minimize objectionable residue formation, as well as of agents effective to lower or raise the temperature of the generated gases. It is further apparent that the proportion of the phenol sensitizer relative to the guanidine nitrate 70 may vary widely depending upon various factors such, for example, as the working pressure at which the charge is intended to operate, the presence or absence of decomposition-assisting or promoting agents, how much (if any) diluent or heat-absorbing volatilizable material is employed in combination with the gas-generating charge.

proper for dispersion thereby, and so on, the proportion of sensitizer increasing with lowering of such working pressure, and being also necessarily greater where such volatilizable material is associated with said charge proper.

It is an advantage of the invention that the novel compositions may be made by simple admixture of the ingredients, and that when the charge is required to be of compact structure and predetermined form so that it will react only on its exposed external surface, it may be made by compressing the mixture into a mold of the desired shape. Moreover, if it is required to protect a portion of the surface of the compact charge from the hot gases evolved by means of an adherent covering of heat-insulating material, this may if desired be done in the course of the pressing operation of applying protective material to the surface of the charge after it has been shaped.

The gas-producing mixtures of the present invention undergo decomposition much more slowly than do black-powder compositions, for example, and hence are safer to handle. Moreover, the gases can be produced at temperatures on the order of 1000° C., which is relatively low for propellant compositions, rendering them particularly well suited for use in driving engines. Under comparable conditions, gases generated from guanidine nitrate sensitized by nitrocellulose (as heretofore proposed) are much hotter than this, sometimes too hot to use for driving engines.

It is also to be observed that the compositions of the invention can be pressed into tubes and thereby obtain layer-by-layer combustion, without any danger of the compressed charges breaking up and exposing uncontrollable burning surfaces. Again, as hereinabove illustrated, 99% of the charge can be converted into gaseous products, leaving behind only about 1 per cent residue which, moreover, is not entrained in the gases. Furthermore, although the temperature of propellant gases can be higher for rockets than for engines, the invention provides novel charge compositions that can be advantageously employed in rockets because said compositions can be used at relatively low pressures, thus requiring only light casings for such rockets.

When the rate of gas evolution is not to be controlled, as may often be the case where a diluent to be dispersed (e. g. a pesticide) is included in the charge, the novel compositions may be employed in loose powder form instead of being compressed into pellets. The ingredients of the novel compositions are all dry materials except that a small amount of liquid, on the order of 1 per cent or thereabouts, may be included, for example mineral oil (see Example 2 hereinabove), to reduce dusting where some or all of the ingredients are in finely powdered form.

In the most desirable embodiments of the invention, the two indispensable components of the novel gas-generating charges, namely, guanidine nitrate and the decomposition-assisting phenol, together constitute at least 75 to 80 per cent of the whole charge, whether or not the charge includes diluent material of the character hereinabove pointed out. Where such diluent is absent, these two components most desirably constitute at least 90 to 95 per cent or more of the charge. In Examples 1 and 2 given hereinabove which represent charge compositions that are highly satisfactory where maximum production of clean power gases is the primary objective, somewhat more than 98 per cent of each of the described charges consists of said two components, the proportion of the phenol approximating 10 per cent of the charge in both instances.

This application is a continuation-in-part of the present applicant's prior application Serial No. 42,948, now abandoned, filed August 6, 1948, and copending herewith. All subject matter contained in said prior application is to be regarded as included herein by reference.

What is claimed is:

1. A non-explosive gas-generating charge consisting in major part of guanidine nitrate and comprising admixed therewith, in proportion not exceeding 35 per cent by weight thereof, a phenol containing in addition to at least one phenol hydroxyl group a plurality of substituent groups each consisting of a nitrogen atom attached exclusively to at least one terminal oxygen atom and to one of the nuclear carbon atoms of the phenol; said charge being non-detonatable by a blasting cap and being capable, when a localized portion thereof is heated sufficiently hot to initiate decomposition, of self-sustaining, non-detonating, gas-evolving, exothermic decomposition at pressures lower than 70 atmospheres.
2. A non-explosive gas-generating charge as claimed in claim 1, wherein guanidine nitrate constitutes at least 60 per cent of the charge by weight.
3. A non-explosive gas-generating charge as claimed in claim 2, wherein the proportion of the phenol employed is from about 5 per cent to about 30 per cent by weight of the guanidine nitrate.
4. A non-explosive gas-generating charge as claimed in claim 1, wherein the guanidine nitrate constitutes at least about 65 per cent of the charge by weight and wherein the proportion of the phenol employed is from about 5% to about 30% by weight of the guanidine nitrate.
5. A non-explosive gas-generating charge as claimed in claim 4, wherein the guanidine nitrate and the phenol together constitute at least about 75 per cent of the charge.
6. A non-explosive gas-generating charge as claimed in claim 1, wherein the guanidine nitrate and the phenol together constitute at least 90 per cent of the charge, and which further includes not to exceed 5 per cent of non-volatile material capable of acting catalytically to promote maximum production of gases in said decomposition, said non-volatile material being selected from the group consisting of vanadium oxides and vanadium compounds thermally decomposable to yield vanadium oxides, metallic molybdenum, molybdic acid, molybdic oxide and ammonium molybdate.
7. A non-explosive gas-generating charge as claimed in claim 6, wherein the guanidine nitrate and phenol together constitute approximately 98 per cent of the charge.
8. A non-explosive gas-generating charge as claimed in claim 7, wherein the phenol is 2:4 dinitroresorcinol and constitutes approximately 10 per cent of the charge, said charge also including up to 1 per cent each of vanadium pentoxide and asbestos fibre.
9. A non-explosive gas-generating charge capable of self-sustained, exothermic non-detonating, flameless, decomposition at relatively low pressure upon heating a localized portion thereof to incipient active decomposition temperature, which charge consists in major part of guanidine nitrate and further includes an admixed compound selected from the group consisting of 2:4 dinitroresorcinol, 2:4:6 trinitro-resorcinol, 2:4 dinitroso-resorcinol, 4:6 dinitro-orthocresol, 3:5 dinitro-catechol, 2:6 dinitro-para-cresol, and 3:5 dinitro-salicylic acid, the proportion of such admixed compound being from about 3 to about 35 per cent by weight of the guanidine nitrate component.
10. A gas-generating charge as claimed in claim 9, wherein said admixed compound is 2:4 dinitro-resorcinol.
11. A gas-generating charge as claimed in claim 9, wherein said admixed compound is 2:4 dinitro-catechol.
12. A gas-generating charge as claimed in claim 9, wherein said admixed compound is 2:4 dinitroso-resorcinol.
13. A gas-generating charge as claimed in claim 9, wherein said admixed compound is 4:6 dinitro-ortho-cresol.
14. A gas-generating charge as claimed in claim 9, wherein said admixed compound is 3:5 dinitro-salicylic acid.

15. A non-explosive gas-generating charge as claimed in claim 1, wherein a portion only of such phenol is replaced by an aliphatic carboxylic acid in amount not exceeding 10 per cent of the charge by weight, said carboxylic acid being selected from the group consisting of tartaric, maleic, citric and fumaric acids.

16. A non-explosive gas-generating charge as claimed in claim 1, wherein the guanidine nitrate constitutes at least about 60 per cent by weight of the charge, and the proportion of the phenol is from about 5 per cent to about 30 per cent by weight of the guanidine nitrate; which charge further includes not more than about 5 per cent of non-volatile heat-resistant solid material capable of acting catalytically to promote maximum production of gases in said decomposition, said solid material being selected from the group consisting of vanadium oxides and vanadium compounds thermally decomposable to yield vanadium oxides, metallic molybdenum, molybdc acid, molybdc oxide and ammonium molybdate.

17. A non-explosive gas-generating charge as claimed in claim 16, wherein the charge further includes a small proportion of potassium nitrate not exceeding 5 per cent by weight.

18. The combination, with the charge defined in claim 1, of a container confining said charge and provided with a gas-discharge outlet, of a gas-permeable body of non-volatile, solid, heat resistant filamentary catalytically active large-surface contact material interposed between said charge and said outlet, through which gases resulting from decomposition of said charge are compelled to pass en route to said outlet.

19. The combination claimed in claim 18, wherein said material is selected from the group consisting of iron, steel, platinum, asbestos.

20. A non-explosive gas generating charge as claimed in claim 1, wherein the guanidine nitrate and the phenol together constitute at least 90% of the charge, and which further includes not more than 2% by weight of the charge of a non-volatile heat-resistant catalytically active filamentary, large-surface contact material.

21. A non-explosive gas-generating charge as claimed in claim 20, wherein said large surface contact material is selected from the group consisting of iron, steel, platinum, and asbestos.

22. A non-explosive gas generating charge as claimed in claim 1, wherein the guanidine nitrate and the phenol together constitute at least 90% of the charge, which further includes not more than 2% by weight of the charge of a non-volatile heat-resistant catalytically active filamentary, large-surface contact material, and a small proportion of potassium nitrate not exceeding 5% by weight.

23. A non-explosive gas generating charge as claimed in claim 22 wherein the proportion of potassium nitrate is from 0.25% to 1%.

References Cited in the file of this patent

UNITED STATES PATENTS

|    |           |        |                |
|----|-----------|--------|----------------|
| 25 | 899,855   | Abelli | Sept. 29, 1908 |
|    | 2,195,965 | Holm   | Apr. 2, 1940   |

FOREIGN PATENTS

|    |         |               |              |
|----|---------|---------------|--------------|
| 20 | 21,529  | Great Britain | 1905         |
|    | 26,430  | Great Britain | 1907         |
|    | 583,986 | Great Britain | Jan. 3, 1947 |